

# United States Patent Office

3,153,604

Patented Oct. 20, 1964

1

3.153.604

3,155,604

**AMMONIUM NITRATE PROPELLANT COMPOSITION CONTAINING NITRILOTRIACETATE**

TION CONTAINING NITROGLUTACETATE  
Wayne A. Proell, Chicago, and Edwin F. Morello, Joliet,  
Ill., and Gavin H. Peters and Walter W. Butcher,  
Hammond, Ind., assignors to Standard Oil Company,  
Chicago, Ill., a corporation of Indiana  
No Drawing. Filed Feb. 23, 1962, Ser. No. 175,354  
5 Claims. (Cl. 149—19)

**5 Claims. (Cl. 149—19)**

This invention relates to ammonium nitrate compositions suitable for use as gas generating materials and particularly having propellant utility. More particularly the invention relates to an ammonium nitrate propellant characterized by substantial independence of the burning rate with combustion chamber pressure.

Ammonium nitrate compositions suitable for use as gas generating materials, and particularly the larger shaped configurations used as propellants are pressure sensitive with respect to the burning rate of the composition. Up to this time ammonium nitrate compositions made up of ammonium nitrate, oxidizable organic material, and a combustion catalyst have exhibited an increase in the burning rate, inches per second of a strand burning cigarette fashion, with increasing pressure in the combustion chamber. It is difficult to prepare shaped ammonium nitrate propellants which are absolutely homogeneous and uniform in composition. These imperfections result in small changes in burning rate and changes in pressure in the combustion chamber. Also in the large rocket motors, it is difficult to maintain chamber pressure absolutely constant over a prolonged burning period. The usual variation in burning rate with pressure variation is sufficient to affect the accuracy of a ballistic missile. A composition which showed substantially no burning rate variation over even a narrow pressure range would be of inestimable value to rocketry.

An ammonium nitrate composition has been discovered which exhibits no burning rate variation substantially within the error of determination of such rates over combustion chamber pressure variation range of as much as 500-600 p.s.i. This "flat" burning rate occurs in a pressure range which is of particular usefulness in propulsion applications, namely, in the region of 1000-1600 p.s.i. combustion chamber pressure.

The solid propellant composition of the invention consists of:

| Component—                                                                                                             | About, weight percent |
|------------------------------------------------------------------------------------------------------------------------|-----------------------|
| Cellulose acetate                                                                                                      | 7-10                  |
| Acetyl triethyl citrate                                                                                                | 7-10                  |
| Dinitrophenoxyethanol                                                                                                  | 7-10                  |
| Alkali metal aminobenzoate                                                                                             | 1-4                   |
| Finely divided carbon                                                                                                  | 3-5                   |
| Ammonium oxalate                                                                                                       | 0.5-2                 |
| Ammonium nitrilotriacetate                                                                                             | 1-2                   |
| Aromatic hydrocarbon amine gassing inhibitor                                                                           | 0.5-1.5               |
| Phenylmorpholine                                                                                                       | 0.5-1                 |
| $\text{RNH}(\text{CH}_2)_x\text{NH}_2$ where R is alkyl having about 8-20 carbon atoms and x is an integer from 2 to 4 | 0.1-0.5               |
| Nonionic surfactant                                                                                                    | 0.0-0.6               |
| Ammonium nitrate                                                                                                       | Remainder             |

The term "ammonium nitrate" as used in this specification and in the claims is intended to mean either C.P. grade or ordinary commercial grade ammonium nitrate or military grade. The particles may be coated with a small amount of moisture-resisting material such as paraffin or petro-latum or paraffin. A minor amount of other inorganic nitrates such as sodium nitrate and/or potassium nitrate

2

may be present. Finely ground ammonium nitrate is preferred.

The combustion catalyst utilized in the composition of the invention is an alkali metal salt of aminobenzoic acid. The sodium salt of ortho aminobenzoic is preferred. Hereinafter, the preferred salt is identified by the trivial name, sodium anthranilate.

The composition of the invention includes in its content of oxidizable organic material, as a cooling material, an ammonium oxalate and preferably diammonium oxalate.

The composition of the invention includes an oxidizable material functioning as a stabilizer. This stabilizer is a salt of a nitrogen base and nitrilotriacetic acid; preferably the stabilizer is ammonium nitrilotriacetate.

15 The composition of the invention also includes phenylmorpholine, which may be the pure compound or commercial technical grade material.

Further, the composition includes an N-alkyl substituted polymethylene diamine where the alkyl substituent which has 8-20 carbon atoms, and the number of methylene groups are 2-4. This diamine may be represented by the formula  $RNH(CH_2)_xNH_2$  where R is alkyl and has 8-20 carbon atoms and x is an integer from 2-4. It is preferred to utilize the N-alkyl substituted 1,3-propylene diamines where the alkyl substituent contains 14-18 carbon atoms. This class of diamines is available commercially under the trade name "Duomeen." A particularly suitable material is that available as "Duomeen T" which has the 1,3-propylene diamine backbone with the N-alkyl substituent derived from tall oil fatty acids.

35 The composition of the invention includes as a burning rate accelerator finely divided carbon. The carbon component of the propellant composition includes finely divided, highly adsorptive activated carbons. These are well known in the art of decolorizing sugar and adsorption of gases. Examples of these are "Norit" and "Nuchar," the former being a high-adsorptive activated carbon used to absorb odors, and to decolorize water, gases, chemical solutions, oils and greases. Nuchar is an activated carbon made from a residual organic material obtained in the manufacture of cellulose and is characterized by high porosity resulting in high adsorptive capacity. Like "Norit" it is used as a decoloring and deodorizing agent.

45 A second general class of carbon useful for increasing the burning rate of the propellant composition are the carbon blacks. These are roughly classified as channel blacks prepared by the impingement of small natural gas flames, furnace combustion blacks produced by the partial combustion of essentially gaseous hydrocarbons in closed retorts and furnace thermal blacks produced by thermal decomposition of hydrocarbons such as acetylene in preheated furnaces. The carbon blacks are characterized by low ash content by having extremely small particle size, that is, 50 to 5000 Å, and contain adsorbed hydrogen and oxygen. Other carbon blacks which may be used in the propellant grains are lamp blacks produced by burning liquid fuels such as petroleum oils, tars and aromatic residues in specially designed pans, combustion taking place under restricted air supply conditions. The carbon blacks as indicated above are generally characterized by exceedingly small particle size, that is, well below #325 U.S. Standard sieve particle size. However, to avoid dusting and convenience in handling, some carbon blacks are formed to the so-called "bead" type carbon blacks which "beads" are generally of such dimensions as to pass through a #20 U.S. Standard sieve and are retained on a #200 U.S. Standard sieve. The "beads" are very soft and are physically unstable as beads and become disintegrated to smaller than #325 U.S. Standard sieve during the mixing and milling of the composited

propellant components as described hereinbelow. The carbon blacks are of low ash content, and usually contain less than 0.5% ash. Examples of "bead" type carbon blacks are Micronex Beads (channel blacks) and Statex Beads (furnace blacks).

A third type of carbon which is useful for improving the burning rate of our gas-producing propellant composition is graphite, flake and amorphous. If desired from a natural graphite, the ash content should be reduced below about 5% which can be accomplished by treating the natural product by air flotation or the ash content may be reduced by leaching with mineral acid or by other methods well known to the art. We prefer graphite of colloidal or semi-colloidal particle size.

Still another type of carbon which we have found effective for increasing the burning rate of the gas-forming composition is finely ground petroleum coke, particularly petroleum coke obtained as a residue in the pipe-stilling of Mid-Continent heavy residuum. Such coke usually contains less than about 1% ash and is preferably pulverized to pass through a #325 U.S. Standard sieve prior to incorporation in the gas-producing propellant composition. The coke may be activated by methods well known to the art to improve the efficiency thereof as a burning rate promoter in our propellant composition.

Ammonium nitrate compositions in general tend to develop gas in storage at elevated temperatures. The composition of the invention includes a gassing inhibitor component. Aromatic amines when introduced into the ammonium nitrate based grain containing catalyst and finely divided carbon have the very desirable characteristic of decreasing the amount of gassing in high temperature storage and frequently even eliminating or essentially eliminating gassing for prolonged periods of time. The aromatic amine gassing inhibitors of this invention are illustrated by diphenylamine, dinaphthylamine and phenyl naphthylamine. In the case of the naphthyl amines, the linkage between the naphthyl radical and the nitrogen may be either alpha or beta. And those amines represented by the empirical formula



In this empirical formula Z is an aromatic nucleus selected from the class consisting of phenyl and naphthyl; R is selected from the class consisting of hydrogen and alkyl containing from 1 to 12 carbon atoms; R' and R'' are selected from the class consisting of hydrogen, and alkyl containing from 1 to 4 carbon atoms; and x is an integer from 1 to 3.

Examples of monoamino-containing compounds are: aniline (monophenylamine, monoamino benzene), 1-naphthylamine, toluidine (methyl aniline) xylidine (dimethylaniline), dodecyl aniline, N-methyl aniline, N,N-dimethyl aniline, N-sec-butyl aniline.

Examples of the diamino compounds are: diamino benzene (phenylene diamine), diamino toluene (toluene diamine), diamino naphthylene, methyl diamino naphthylene, dodecyl diamino naphthylene, N-sec-butyl, diamino benzene, N,N'-di-sec-butyl diamino benzene, and N-methyl diamino naphthylene.

Examples of triamino compounds are: triamino benzene, triamino naphthylene, triamino toluene, and triamino methyl naphthylene.

The composition of the invention may include one or more nonionic surfactants which tend to improve mixing of the composition and molding of shaped configurations. Any nonionic surfactant which is inert to the other components of the composition is suitable for use in the composition. For purposes of illustration, only certain broad classes of nonionic surfactants are set out hereinafter.

The surfactant polymers of alkylene oxides may be the polymers of ethylene oxide, copolymers of ethylene oxide and propylene oxide or block polymers of propylene oxide

and ethylene oxide wherein ethylene oxide is added to polymers of propylene oxide. These polyalkylene oxide condensation products are otherwise known as polyoxyalkylene glycols and have from two to three carbon atoms in the oxyalkylene unit.

One class of the polyoxyalkylene glycols which are effective are the commercial "Pluronics" which are polyoxypropylene-polyoxyethylene glycols or specifically, block copolymers. Pluronic L-62 has a molecular weight of about 2,000 of which 2,000 molecular weight from about 1500 to about 1800 is furnished by the propylene oxide units, the other alkylene oxide units in the polymer molecule being ethylene oxide units. The general formula for the Pluronics is



Thus "b" in this formula, for Pluronic L-62, has a value of about 26 to about 31. Pluronic L-62 is a liquid having a viscosity at 25° C. of 300 to 500 centipoises.

As indicated hereinabove, derivatives of the polyoxyalkylene glycols are effective to reduce the consistency of the ammonium nitrate-binder mixtures. Certain of these derivatives are the fatty alcohol monoethers and the fatty acid monoesters. An example of the monoether derivative is Tergitol XC. Tergitol XC is a monoether derivative of a copolymer of ethylene oxide and propylene oxide and has the approximate formula



wherein R is an acyclic hydrocarbon radical containing from 12 to 20 carbon atoms. The alkylene oxide constituents of the molecule each contribute about 1500 to give about 3000 to the total molecular weight, i.e., not more than about 3300, of the monoether derivative. In these ether derivative-type surfactants the number of ethylene oxide units may vary from about 22 to 35 and the number of propylene oxide units may vary from about 18 to about 27. The total molecular weight of these ethers will usually lie within the range of from about 2000 to about 3300.

An example of a monoester derivative of a polyoxyalkylene glycol which is effective is the commercial product "Nonisol-250." This product is a mono-oleyl ester of polyoxyethylene having a molecular weight of about 1000. The fatty acid esters of polyoxyethylene sorbitol condensation products are effective surfactants for purposes of this invention. These may be produced by condensing ethylene oxide or polyoxyethylene with sorbitol followed by esterification of the condensation product with a 12 to 20 carbon atom fatty acid. In general, suitable products of this type have molecular weights within the range of from about 1000 to about 3300.

The term "polyoxyalkylene glycol, ether and fatty acid ester derivatives thereof," as used in this specification and claims includes (1) the polyethylene oxide homopolymers, copolymers or ethylene oxide and propylene oxide, block copolymers or propylene oxide and ethylene oxide, said polymers having a molecular weight within the range of from about 1000 to about 3000, (2) the monoethers of the polymers of (1) produced by reacting fatty alcohols and mercaptans having 10 to 20 carbon atoms with polymers of (1) said ethers having a molecular weight of about 2000 to about 3300, and (3) monoesters of the polymers of (1) produced by esterification of said polymers with fatty acids having from 12 to 20 carbon atoms per molecule, said monoesters having molecular weights within the range of about 1000 to about 3300. The fatty acids used to esterify the condensation product of ethylene oxide with sorbitol have from 12 to 20 carbon atoms, and the fatty acid esters produced have molecular weights within the range of from about 1000 to about 3300.

Particularly effective are the nonionic surfactants which may be classified as esters of monoanhydro sorbitols described in U.S. 2,398,193. These are known commercially as the "Span" and "Arlacel" described on page 3

of a brochure entitled "Atlas Surface Active Agents," is issued in 1950. The sorbitans are mixtures of cyclized monoanhydized sorbitol. The preferred Span materials for use in the composition are essentially partial esters of oleic acid and sorbitol monoanhydrides (sorbitans) derived from sorbitol, the sorbitan oleates being mixtures containing an average of from 1 to 3 oleyl radicals for each molecule of anhydized sorbitol. Sorbitol is dehydrated to give condensed link structures or sorbitans which, when esterified with oleic acid, produce the preferred Spans or Arlaces. Arlace C, which is sorbitan sesquioleate, has been found to be particularly effective as an additive to promote ballistic dependability of the grain compositions. This material is an oily liquid at 25° C. having a specific gravity of 0.95-1.00, a flash point of about 450° F. and a fire point of about 530° F.

Arlace C has a viscosity at 25° C. of 900-1100 centipoises. Another very effective nonionic surfactant is Span 85, which is a sorbitan trioleate having a viscosity at 25° C. of 100-250 centipoises. It has a specific gravity of 0.92-0.98, a flash point of 500° F. and a fire point of 570° F.

With the exception of the hereinabove defined combustion catalyst and the ammonium nitrate, the other components of the composition may be considered as oxidizable organic materials. In a narrower sense, organic materials are present to function as a binder for the ammonium nitrate catalyst and other solid components. The binder material utilized in the instant composition consists of cellulose acetate, acetyl triethyl citrate and dinitrophenoxethanol.

The acetyl triethyl citrate is a well known plasticizer. The citrate may be the pure compound or commercial technical grade.

The dinitrophenoxethanol component may be essentially pure material, or more usually will be a mixture of one or more of the dinitrophenoxethanols and a bis-(dinitrophenoxo)ethane. In all cases, the dinitrophenoxethanol is the predominant member and usually will represent 70% or more of this component. A mixture of 2,4-dinitrophenoxethanol and 1,2-bis-(2,4-dinitrophenoxo)ethane is particularly suitable. U.S. Patent No. 2,935,415 at columns 2 and 3 sets out a description of classic methods of preparation of the mixture of the two materials and the separation thereof. U.S. Patent No. 2,988,571 sets out a method of preparation of high purity dinitrophenoxethanol.

The polymeric material present in the binder is cellulose acetate. Particularly suitable are the cellulose acetates which have combined acetic acid contents on the order of 50-58%. A preferred cellulose acetate is one made by the Celanese Company as grade HLFS-93, which has a combined acetic acid content of about 55%.

#### Examples

Two illustrative examples of the results obtainable in terms of uniformity of burning rate with variation of pressure are set out. The burning rate-pressure results set out below were obtained by burning a strand at a given pressure in the well known Crawford bomb test wherein a strand of a definite shape is burned at a given temperature and pressure, and the burning rate, cigarette fashion, is obtained. In these tests two batches of propellant composition containing the identical percentage of each component were prepared. Each batch represented approximately 20 quarts U.S. of propellant composition. While the component percentages were identical, the conditions of blending were varied between the two batches in order to observe whether or not the composition would give a flat burning rate plateau of its burning rate-pressure curve regardless of the method of blending utilized. It is well known that the burning rate of a propellant composition can be changed by the degree of mixing or the type of mixing used in the prepa-

ration of the composition. This composition follows this same pattern as is shown in the burning rate data below. The data do establish that the degree of mixing has no bearing on the flat burning rate characteristic of the composition.

In general, the blending operation utilized in the preparation of the two batches of propellant utilized in the burning rate tests follows that of the prior art, such as described in U.S. Patent No. 2,987,388 of William G. Stanley, assigned to Standard Oil Company (Indiana).

The propellant utilized in these tests contained the following materials.

| Component:                                            | Percent by weight |
|-------------------------------------------------------|-------------------|
| Cellulose acetate (cellulose HLFS-93)                 | 8.91              |
| Acetyl triethyl citrate                               | 8.91              |
| Dinitrophenoxethanol                                  | 8.12              |
| Sodium anthranilate                                   | 2.00              |
| Carbon black                                          | 4.00              |
| Ammonium oxalate                                      | 1.00              |
| Ammonium nitrilotriacetate                            | 0.90              |
| Toluene diamine                                       | 0.50              |
| Phenylmorpholine                                      | 0.50              |
| Duomeen T                                             | 0.10              |
| Arlace C (sorbitan sesquioleate)                      | 0.10              |
| Nonic 259 (polyethylene glycol tertdodecyl thioether) | 0.03              |
| Ammonium nitrate (Spencer C.P.)                       | 64.93             |

The burning rate data obtained for the two batches are set out below.

| Pressure (p.s.i.) | Batch 1 | Batch 2 |
|-------------------|---------|---------|
| 600               | 0.55    | 0.50    |
| 1,000             | 0.75    | 0.67    |
| 1,100             | 0.76    | 0.68    |
| 1,200             | 0.77    | 0.68    |
| 1,300             | 0.78    | 0.69    |
| 1,400             | 0.78    | 0.69    |
| 1,500             | 0.78    | 0.70    |
| 1,600             | 0.79    | 0.74    |
| 1,700             | 0.80    | 0.76    |
| 2,000             | 0.86    | 0.82    |

The above data establish that batch No. 1 shows essentially no variation in burning rate beyond the error of determination of these rates over the region 1000-1600 p.s.i. Batch No. 2 shows essentially no variation in burning rate over the range of 1000-1500 p.s.i. It is considered that the difference in burning rate at the standard pressure of 1000 p.s.i. is normal for the difference in mixing technique—herein the severity of the blending operation—known to exist between the two batches of propellant.

Thus having described the invention, what is claimed is:

1. A solid composition consisting of cellulose acetate, about 7-10%; acetyl triethyl citrate, about 7-10%; dinitrophenoxethanol, about 7-10%; alkali metal amino-benzoate, about 1-4%; finely divided carbon, about 3-5%; ammonium oxalate, about 0.5-2%; ammonium nitrilotriacetate, about 1-2%; aromatic hydrocarbon amine gassing inhibitor, about 0.5-1.5%; phenylmorpholine, about 0.5-1%; a diamine of the formula



where R is alkyl having about 8-20 carbon atoms and x is an integer from 2 to 4, about 0.1-5%; a nonionic surfactant, about 0.0-0.6%; and the remainder of said composition being essentially ammonium nitrate, said gassing inhibitors are selected from the class consisting of diphenylamine, dinaphthylamine, phenyl naphthylamine and  $RZ(NR'R'')_x$  where Z is an aromatic nucleus selected from the group consisting of phenyl and naphthyl; R is selected from the group consisting of hydrogen and alkyl containing from 1 to 12 carbon atoms; R' and R'' are selected from the group consisting of hydrogen, and alkyl containing from 1 to 4 carbon atoms; and x is an integer from 1 to 3.

2. The composition of claim 1 wherein said gassing inhibitor is toluene diamine.

3. The composition of claim 1 wherein said diamine is an N-alkyl propylene diamine where the alkyl substituent is derived from saturated tallow fatty acids.

4. The compositions of claim 1 wherein said surfactant is sorbitan sesquioleate.

5. A solid composition consisting of cellulose acetate, about 9%; acetyl triethyl citrate, about 9%; dinitro-phenoxyethanol, about 8%; sodium anthranilate, about 2%; carbon black, about 4%; diammonium oxalate, about 1.0%; ammonium nitrilotriacetate, about 1%; toluene diamine gassing inhibitor, about 0.5%; phenyl-

morpholine, about 0.5%; a diamine of the formula  $RNH(CH_2)_xNH_2$  where R is alkyl having 14-18 carbon atoms and x is 3, about 0.1%; sorbitan sesquioleate, about 0.1%; polyethylene glycol tertdodecyl thioether, about 0.03%; and the remainder of said composition being ammonium nitrate.

References Cited in the file of this patent

UNITED STATES PATENTS

|    |           |                 |       |               |
|----|-----------|-----------------|-------|---------------|
| 10 | 2,938,778 | Linsk           | ----- | May 31, 1960  |
|    | 2,942,964 | Burgwald et al. | ----- | June 28, 1960 |
|    | 2,946,671 | Marti           | ----- | July 26, 1960 |
|    | 2,973,255 | Eiszner         | ----- | Feb. 28, 1961 |